

May 3, 1932.

O. H. HERTEL

1,856,252

## PROCESS OF CARBONIZING COAL

Filed Dec. 4, 1925



Inventor:

Otto H. Hertel  
By Chindall Parker Tolson  
(Atty.5.

## UNITED STATES PATENT OFFICE

OTTO H. HERTEL, OF CHICAGO, ILLINOIS

## PROCESS OF CARBONIZING COAL

Application filed December 4, 1925. Serial No. 73,171.

This invention relates to the production of a fuel of novel and desirable characteristics through the carbonization of bituminous coal and the like.

6 Coke produced by carbonizing coal at high temperatures is very porous, and because of the great extent of surface it burns rapidly and produces an intense heat. This is also true of coke produced in an experimental way 10 by the various methods heretofore proposed of carbonizing coal at relatively low temperatures.

In the production of high-temperature coke and in the production of coke by 15 previous methods of so-called low-temperature carbonization, a larger percentage of the volatile constituents of the coal has been driven off than is desirable in domestic fuel.

The low density of the product and the 20 relatively small percentage of volatile material remaining therein have been due partly to the use of temperatures in excess of that at which exothermic reactions will be useful in the coal, and partly to the fact that while the 25 material was plastic it was free to expand as gas was being evolved therefrom. I have discovered that if only sufficient heat be applied to the coal to initiate exothermic reaction within the coal, and if the material be 30 maintained under pressure while plastic, the product will be substantially without pores and hence relatively dense, will contain a relatively large percentage of volatile material, will burn with moderate intensity, and 35 will not produce clinkers.

When a typical variety of bituminous coal is placed in a retort and the retort subjected to sufficient heat to raise the temperature of the contents to about 390° C., exothermic 40 action occurs in the coal, the temperature rising slightly and then subsiding as the reaction is completed, gas and vapors being meanwhile liberated. The char resulting from this reaction is deep black in color and 45 has a vitreous luster. If the char thus produced be raised to a temperature of about 475° C., additional exothermic reaction occurs with the evolution of gas and vapors, the color of the char changing to a gray black 50 and having, when struck, a metallic ring of

higher pitch than that of the char first produced.

Certain methods heretofore used in carbonizing coal at relatively low temperatures have resulted in the production of an excessive percentage of breeze. In order to dispose of the breeze and to improve the strength of the coke, the breeze has been mixed with raw coal in varying proportions. As will readily be understood, the passing of 55 a large percentage of the product through the retort a second time increases the expense of treatment to a substantial extent.

In view of the fact that the term "low-temperature coke" is very indefinite as to the 60 character of the material carbonized, the temperature employed, and the density, structure, hardness, color, luster and volatile content of the product, I shall hereinafter use the more general term "char".

The object of the present invention is the 65 production of a fuel which shall be sufficiently hard and strong so as not to be subject to excessive degradation in handling, which shall be sufficiently dense so that it may be shipped economically and so that it shall not burn with excessive intensity, which shall contain a relatively large percentage of volatile matter, and which shall not form 70 clinkers.

The invention also aims to provide a method of carbonizing coal whereby the product shall be uniform in quality and whereby the 75 production of an excessive percentage of breeze shall be avoided.

While some of the desirable results just mentioned may perhaps be attained in some form of continuous process, I believe that the greatest degree of efficiency can be obtained 80 in a batch process which will allow the material to be at rest while it is setting, and which will permit of maintaining pressure upon the material while it is plastic and while undergoing the change from plasticity to rigidity. I have therefore selected for illustration two 85 forms of apparatus wherein the material may be treated in batches, as distinguished from apparatus through which the material moves continuously as a stream.

In the accompanying drawings, Figure 1 100

is a vertical sectional view of one form of apparatus by means of which my improved process may be practiced.

Fig. 2 is a transverse sectional view of a 5 rotor comprised in said apparatus.

Fig. 3 is a longitudinal sectional diagrammatic view of another form of apparatus which may be used in producing said fuel.

For a detailed description of the apparatus shown in Fig. 1, reference may be made to my application Serial No. 699,402, filed March 15, 1924. It will be sufficient here to say that 10 denotes a vertical elongated retort which is relatively narrow in one direction, say, about thirty inches in width. The retort has a slight taper inwardly toward the top to facilitate the discharge of char downward. Any preferred form of furnace, as, for example, the furnace 12, may be used to 15 apply heat to the exterior of the retort. At the lower end of the retort are discharge chutes 26 which are closed in any preferred manner, as by means of trap doors 27. 28 denotes a bottom for the retort, said bottom 20 being arranged to be lowered from the normal position shown in dotted lines to that shown in full lines when the contents of the retort are to be discharged.

A feed hopper 30 communicates with the 30 upper end of the retort and is provided with a trap door 31. An upwardly tapering weight 32 is movable up and down within the retort, the weight being shown in charging position in full lines in Fig. 1. The granular 35 or powdered coal being charged into the retort is compelled to pass down through a relatively narrow space between the weight and the retort wall in the form of a thin stream or layer, which in falling exposes the grains 40 and small lumps of coal to the heat of the retort, thus causing a rapid and uniform heating of the coal before the same is deposited at rest, which substantially reduces the time consumed in carbonizing the charge. 45 When the retort is fully charged the weight 32 is lowered onto or pressed against the material by any preferred means, as, for example, the hydraulic cylinder 35, the piston 36 of which is connected to said weight by 50 means of a piston rod 33, cross head 33<sup>a</sup> and rods 34. By this means the weight can be raised or lowered as well as adjusted to resist yieldingly the pressure of the swelling charge, to place pressure upon the mass while 55 plastic, and to discharge the char at the end of the operation.

The gases and vapors evolved from the charge are withdrawn through a pipe 40 communicating with the upper end of the retort.

60 Within the retort is rotatably mounted a tubular member 44. A thirty-inch retort would have a rotor of approximately twelve inches in diameter. While the rotor may be cylindrical and mounted to rotate upon its 65 central axis, the rotor is preferably of such

cross-sectional form as to exert pressure upon the contents of the retort as the rotor turns. Herein the rotor is shown as consisting of a cylindrical tube having a longitudinally extending plate or sole 44<sup>a</sup> secured thereto. The rotor 44 may be rotated in any preferred manner, as, for example, by means of bevel gearing 45.

Means is provided for internally heating the rotor 44. While such means may be of any preferred character, there is herein shown a candle 46 like that fully described in my application Serial No. 28,614, filed May 7, 1925. The candle is supplied with gas by means of pipes 47 provided with valves 48.

In use, the retort 10 is filled with powdered or granular coal and the weight 32 operated to press against the charge. Heat being applied to the outside of the retort 10 and to the interior of the rotor 44, the charge is rapidly heated, the entire mass being substantially uniformly raised in temperature by reason of the application of heat both externally and internally, and through the action of the rotor. The latter serves to distribute heat to the charge, since the coal will follow the eccentric portion of the rotor, thus causing agitation of the coal. Friction among the solid particles likewise conduces to the heating of the charge. Moreover, the rubbing action of the rotor accelerates the delivery of heat into the mass.

As the rotor turns it forms a passage through the central portion of the charge, through which passage the gases and vapors quickly escape from the charge. It will be seen that the material being carbonized is arranged in a relatively thin layer, and that the gases and vapors do not have far to travel in order to emerge from the layer. The layer form of the material undergoing treatment increases the surface exposed to the heat of the retort and the rotor, and thus assists to reduce the time of operation. As the rotor turns the coal moves to fill the constantly shifting gas passage until the stage where the coal becomes plastic is reached. When the mass begins to set there is less and less tendency to close in around the rotor and thus the delivery of heat to the mass from the rotor is in a measure self-regulating, the amount of heat supplied to the mass from the rotor being automatically reduced as the need for the application of heat diminishes.

As the mass becomes plastic, it tends to flow into the shifting gas passage and thus close the latter, but the rotation of the rotor is sufficiently rapid to maintain a passage for the gas. Moreover, in its rotation the rotor exerts lateral pressure on the charge, which assists to impart a desirable density and hardness to the char. Pressure is also exerted upon the contents of the retort by means of the weight 32, whereby the char is rendered relatively dense and hard.

In Fig. 3 is illustrated diagrammatically a form of apparatus comprising a cylindrical retort 50 which is closed at one end by means of a removable cap 51. The opposite end of 5 the retort is closed by a piston 52, by means of which pressure may be placed upon the contents of the retort by operating the screw 53. The latter engages an internally threaded portion 54 carried by a yoke 55 which is 10 pivoted or otherwise suitably secured to the retort so that the piston, when withdrawn, may be swung aside to permit of charging the retort. In the piston 52 are openings 56 for the escape of gases and vapors. The 15 retort 50 having been filled with granular or pulverized coal and pressure having been placed upon the charge by means of the screw 53, the retort may be inserted into any suitable form of furnace. The screw 53 may be 20 operated from time to time to maintain pressure upon the charge. When the mass fuses the piston 52 may be advanced to maintain the mass under pressure, this pressure being maintained until the material has set. The 25 retort may then be withdrawn from the furnace, the cap 51 removed and the char expelled by means of the piston 52 and the screw 53.

In accordance with my process, the heat 30 to which the coal is subjected is just sufficient to fuse the coal and initiate exothermic reactions therein. (In the case of the coals with which I have experimented, the coal is heated to about 390° C.) I thereby reduce 35 the cost of the product by economizing fuel and by shortening the time of treatment. The product also is improved, in that it retains a relatively large percentage (approximately 14%) of volatile matter. By keeping the material under pressure, pores are 40 largely eliminated, the char being relatively dense, hard and strong, the apparent specific gravity of the char being about 1.0. Inasmuch as the material is at rest while it is 45 setting, the char is stronger and harder than char produced by processes which involve movement of the material while it is setting; and there is a very small, practically negligible, percentage of breeze. The entire 50 charge is substantially uniform in character, each lump being substantially like all the other lumps, and each lump being homogeneous or uniform in character throughout. The product is black in color and has a vitreous luster.

By reason of its density and high volatile content, the char produced by the process herein described is particularly well adapted for domestic use. The high volatile content 55 conduces to ease in igniting the fuel, while its density prevents excessively rapid combustion and insures against fusion of the fuel and the production of clinkers.

While the improved fuel herein described is especially adapted for domestic use, it may

also be used in place of ordinary coke in gas-making plants.

I claim as my invention:

1. A process of carbonizing coal that will go through an exothermic reaction accompanied with plasticity upon being heated to a predetermined temperature which consists in heating a definite batch of coal just sufficiently to initiate such exothermic reaction in the batch, and maintaining the batch under 70 mechanical pressure while the batch is plastic and while setting, while allowing gas and vapors to escape, the material being at rest while setting.

2. A process of carbonizing coal that will 80 become plastic when heated to about 400° C. which consists in heating a definite batch of coal just to about 400° C. and maintaining the batch under mechanical pressure until it has set, while allowing gas and vapors to 85 escape freely.

3. A process of carbonizing coal that will 90 become fused when heated to a predetermined temperature which consists in arranging a batch of coal in the form of a relatively thin layer, applying heat to opposite sides of the layer just sufficiently to raise the temperature of the coal to the fusing point, and applying mechanical pressure to the fused material until it has set, while allowing gas and 95 vapors to escape freely.

4. A process of carbonizing coal that will 100 go through an exothermic reaction accompanied with plasticity upon being heated to a predetermined temperature which consists in heating a definite batch of coal just sufficiently to initiate exothermic reaction in the batch, agitating the coal in the batch before plasticity sets in, allowing gas and vapor to escape freely through the center of the batch, 105 yielding restraining expansion of the batch during the exothermic reaction so as to apply pressure thereto while the batch is plastic, and allowing the batch to be at rest while setting.

5. A process of carbonizing coal that will 110 become plastic when heated to a predetermined temperature range, which consists of confining a batch of the coal in a vertical column having a central longitudinal passage therethrough, heating the batch externally and also internally from within said passage just up to said temperature range, agitating said batch while in granular form, and applying mechanical pressure to the top of said 115 batch and to said batch from within said passage while the batch is plastic and while setting, and allowing gases and vapors to escape freely.

In testimony whereof, I have hereunto 125 affixed my signature.

OTTO H. HERTEL.